

F. A. VAUGHN.

PROCESS OF COATING METALS, ALLOYS, OR OTHER MATERIALS WITH PROTECTIVE COATS OF  
METALS OR ALLOYS.

APPLICATION FILED OCT. 5, 1917.

1,281,108.

Patented Oct. 8, 1918.

Fig. 1



Fig. 2



INVENTOR

Francis A. Vaughn

BY

Upson, Peaney & French  
ATTORNEY

# UNITED STATES PATENT OFFICE.

FRANCIS A. VAUGHN, OF MILWAUKEE, WISCONSIN.

## PROCESS OF COATING METALS, ALLOYS, OR OTHER MATERIALS WITH PROTECTIVE COATS OF METALS OR ALLOYS.

1,281,108.

Specification of Letters Patent.

Patented Oct. 8, 1918.

Application filed October 5, 1917. Serial No. 194,942.

*To all whom it may concern:*

Be it known that I, FRANCIS A. VAUGHN, a citizen of the United States, and resident of Milwaukee, in the county of Milwaukee and State of Wisconsin, have invented new and useful Improvements in Processes of Coating Metals, Alloys, or other Materials with Protective Coats of Metals or Alloys, of which the following is a description, reference being had to the accompanying drawings, which are a part of this specification.

The invention relates to a process of coating metals, alloys or other material with a protective or ornamental coating or coatings of metals or alloys.

One of the objects of this invention is to provide a process of coating materials with a metallic coating, more particularly of the non-corrosive varieties, in order to protect such materials from the elements or other destructive chemical and physical agents.

Another object of the invention is to provide a process of coating metals or alloys with a coating of metals or alloys which are dissimilar from the metals or alloys to be coated by interposing a coating of electrolytic insulating material between the metal and its metallic coating to prevent electrolytic action between the dissimilar metals.

I am aware of the fact that numerous attempts have been made to coat materials with metals, either by electro-plating, galvanizing, metallizing or metal spraying, but in all of the above named processes numerous difficulties arise especially with certain metals or combinations of metals, that is, where a layer or layers of dissimilar metal are used as a coat, owing to the fact that in all such methods or processes the object to be coated usually must be thoroughly cleaned by expensive processes such as sand blasting, pickling, etc., and furthermore after the coating has been applied electrolytic or other corrosive action between the dissimilar metals causes reactions which sooner or later cause a failure of the coating, either chemically or physically. The importance of a successful solution of this problem of the elimination of expensive processes of cleaning the materials and the prevention of electrolytic or other corrosive action has long been recognized and the process herein-after described has successfully solved the problem.

My method consists in first coating ma-

terial to be protected with a non-corrosive priming and binder coating and in addition said coating being an electrolytic insulating coating. One material which has all the three properties of forming a priming, 60 binder and electrolytic insulating coating is a solution of alkaline silicate, such as sodium silicate. The material to be protected is thus covered with a coating of a solution of alkaline silicate. This coating of alkaline 65 silicate will cover and seal over the imperfections in the material and the pores of porous material and such detrimental objections as rust, corrosion, or other foreign matter as may exist if the surface to be 70 coated is a metal or alloy. In case the material to be coated is non-metallic the alkaline silicate serves as a priming and binder coating to form a clean binding surface, or matrix, but also forms an elec- 75 trolytic insulating coat to which the protective metal coating can be readily applied.

The next step consists in applying the protective or ornamental coating of metal to the matrix coating. This is done by 80 spraying, impacting or spreading the metal upon the coating. In spraying, the metal is discharged in hot impalpable particles moving with high velocity and these when directed upon the prepared object with the 85 plastic matrix coating applied thereto penetrate said matrix while the spray is still plastic. The coating metal thus dovetails itself into the superficial pores of the matrix coating while the matrix coating binds the 90 metal coating to the object being coated. The plastic matrix coating forms a better binder for the metal coating than can be obtained by spraying the metal directly onto the object to be coated and at the same time forms 95 an electrolytic insulating coat.

If the metal coating applied to the matrix coating is porous, which is generally the case, the object with the coatings applied is then treated so as to render the plastic matrix 100 coating hard and insoluble. When a solution of alkaline silicate is used as a matrix coating it is rendered insoluble by treating the coated object in such a way as to precipitate out the silica as insoluble silicic acid. 105 This may be done in any suitable manner and one way of doing it is to subject the coated object to the action of carbon dioxid either in a gaseous or liquid form. This may be done by placing the coated object in 110

the air, but to hasten the hardening I prefer to expose the coated object to carbon dioxide or a carbon-dioxide-containing atmosphere to allow the carbon dioxide to penetrate through 5 the pores of the metal coating and thus render insoluble any exposed minute areas of the alkaline silicate coat.

In the drawings: Figure 1 is a sectional view showing the protective coating applied 10 thereto in which the outer metallic coating is non-porous; Fig. 2 is a sectional view showing the protective coating applied thereto in which the outer metallic coating is porous.

15 In Fig. 1 the numeral 3 represents the material to be coated, 4 the alkaline silicate coating, and 5 the non-porous metal coating and Fig. 2 shows the material 3 and coating 4 provided with a porous metal coating 6.

20 It is understood, of course, that any combination of alternate coats of alkaline silicate and metal may be used, the last named being either of one kind or each successive coat of a different kind.

25 In case the material to be covered is of a non-metallic character such as wood, glass or fiber, the priming and binding properties of the alkaline silicate are utilized to form a clean binding surface, or matrix, for the re- 30 ception of the protective metal coating.

In case the material to be covered is a corrosive metal or alloy the binding and priming properties of the alkaline silicate are utilized to form a clean binding surface, or 35 matrix, without the necessity of first cleaning the corrosive metal and where the metal coating is of a dissimilar character from that of the metal or alloy being coated the

electrolytic insulating property of the alkaline silicate provides for insulating the two 40 dissimilar metals from each other and thus prevents electrolytic or other corrosive action between them.

What I claim as my invention is:

1. The herein described process of coating 45 metal with a coating of a dissimilar metal which consists in applying a coating of binder and electrolytic insulating material to the metal to be coated, and then spraying molten metal onto said insulating coating to 50 form the protective metal coating.

2. The herein described process of coating metallic material with a metal coating which consists in applying a coating of a solution of alkaline silicate to the material to be 55 coated, and then spraying molten metal onto the aforesaid coating.

3. The herein described process of coating material with a porous metal coating which consists in applying a matrix coating of 60 plastic binder material over the material to be coated, spraying molten metal onto the matrix coating while said matrix coating is in a plastic condition and then hardening the matrix coating.

4. The herein described process of coating material with a porous metal coating which consists in applying a matrix coating of a solution of alkaline silicate to the material to be coated, spraying molten metal onto the 70 matrix coating while said matrix coating is in a plastic condition, and then bringing the material so coated into the presence of carbon dioxide to harden said matrix coating.

In testimony whereof I affix my signature. 75  
FRANCIS A. VAUGHN.